



US007754333B2

(12) **United States Patent**  
**Eyre et al.**

(10) **Patent No.:** **US 7,754,333 B2**  
(b4) **Date of Patent:** **\*Jul. 13, 2010**

(54) **THERMALLY STABLE DIAMOND POLYCRYSTALLINE DIAMOND CONSTRUCTIONS**

4,224,380 A 9/1980 Bovenkerk et al.  
4,255,165 A 3/1981 Dennis et al.

(75) Inventors: **Ronald K. Eyre**, Orem, UT (US);  
**Anthony Griffi**, The Woodlands, TX (US); **Thomas W. Oldham**, The Woodlands, TX (US)

(Continued)

(73) Assignee: **Smith International, Inc.**, Houston, TX (US)

## FOREIGN PATENT DOCUMENTS

EP 0300699 1/1989

(\*) Notice: Subject to any disclaimer, the term of this patent is extended or adjusted under 35 U.S.C. 154(b) by 1116 days.

This patent is subject to a terminal disclaimer.

(Continued)

(21) Appl. No.: **10/947,075**

(22) Filed: **Sep. 21, 2004**

(65) **Prior Publication Data**

US 2006/0060391 A1 Mar. 23, 2006

(51) **Int. Cl.****B32B 9/00** (2006.01)(52) **U.S. Cl.** ..... **428/408**; 51/307; 51/309;

428/325; 428/336; 428/472

(58) **Field of Classification Search** ..... 51/307,

51/309; 428/408, 472, 336, 325

See application file for complete search history.

(56) **References Cited**

## U.S. PATENT DOCUMENTS

|             |        |                     |
|-------------|--------|---------------------|
| 3,136,615 A | 6/1964 | Bovenkerk           |
| 3,141,746 A | 7/1964 | DeLai               |
| 3,233,988 A | 2/1966 | Wentorf, Jr.        |
| 3,745,623 A | 7/1973 | Wentorf, Jr. et al. |
| 4,108,614 A | 8/1978 | Mitchell            |
| 4,151,686 A | 5/1979 | Lee et al.          |

EP 0300699 1/1989

1/1989

Translation of Japanese Unexamined Patent Application No. S59-218500. "Diamond Sintering and Processing Method," Shuji Yatsu and Tetsuo Nakai, inventors; Application published Dec. 10, 1984; Applicant: Sumitomo Electric Industries Co. Ltd. Office Action by USPTO mailed Mar. 11, 2003 for related U.S. Appl. No. 10/065,604.

(Continued)

*Primary Examiner*—Archene Turner(74) *Attorney, Agent, or Firm*—Osha • Liang LLP(57) **ABSTRACT**

Thermally stable diamond constructions comprise a diamond body having a plurality of bonded diamond crystals and a plurality of interstitial regions disposed among the crystals. A metallic substrate is attached to the diamond body. A working surface is positioned along an outside portion of the diamond body, and the diamond body comprises a first region that is substantially free of a catalyst material, and a second region that includes the catalyst material. The diamond body first region extends from the working surface to depth of at least about 0.02 mm to a depth of less than about 0.09 mm. The diamond body includes diamond crystals having an average diamond grain size of greater than about 0.02 mm, and comprises at least 85 percent by volume diamond based on the total volume of the diamond body.

**37 Claims, 6 Drawing Sheets**

# US 7,754,333 B2

Page 2

## U.S. PATENT DOCUMENTS

|               |         |                    |                 |         |                      |
|---------------|---------|--------------------|-----------------|---------|----------------------|
| 4,268,276 A   | 5/1981  | Bovenkerk          | 5,524,719 A     | 6/1996  | Dennis               |
| 4,288,248 A   | 9/1981  | Bovenkerk et al.   | 5,560,716 A     | 10/1996 | Tank et al.          |
| 4,303,442 A   | 12/1981 | Hara et al.        | 5,601,477 A *   | 2/1997  | Bunting et al. ....  |
| 4,311,490 A   | 1/1982  | Bovenkerk et al.   | 5,607,024 A     | 3/1997  | Keith et al.         |
| 4,373,593 A   | 2/1983  | Phaal et al.       | 5,620,382 A     | 4/1997  | Cho et al.           |
| 4,387,287 A   | 6/1983  | Marazzi            | 5,624,068 A     | 4/1997  | Waldenstrom et al.   |
| 4,412,980 A   | 11/1983 | Tsuji et al.       | 5,645,617 A     | 7/1997  | Frushour             |
| 4,481,016 A   | 11/1984 | Campbell et al.    | 5,667,028 A     | 9/1997  | Truax et al.         |
| 4,486,286 A   | 12/1984 | Lewin et al.       | 5,706,906 A *   | 1/1998  | Jurewicz et al. .... |
| 4,504,519 A   | 3/1985  | Zelez              | 5,718,948 A     | 2/1998  | Edervd et al.        |
| 4,522,633 A   | 6/1985  | Dyer               | 5,722,499 A     | 3/1998  | Nguyen et al.        |
| 4,525,179 A   | 6/1985  | Gigl               | 5,776,615 A     | 7/1998  | Wong et al.          |
| 4,534,773 A   | 8/1985  | Phaal et al.       | 5,803,196 A *   | 9/1998  | Fielder ....         |
| 4,556,403 A   | 12/1985 | Almond et al.      | 5,833,021 A     | 11/1998 | Mensa-Wilmot et al.  |
| 4,560,014 A   | 12/1985 | Geczy              | 5,890,552 A *   | 4/1999  | Scott et al. ....    |
| 4,570,726 A   | 2/1986  | Hall               | 5,897,942 A     | 4/1999  | Karner et al.        |
| 4,572,722 A   | 2/1986  | Dyer               | 5,954,147 A     | 9/1999  | Overstreet et al.    |
| 4,604,106 A   | 8/1986  | Hall               | 5,979,578 A     | 11/1999 | Packer               |
| 4,605,343 A   | 8/1986  | Hibbs, Jr. et al.  | 6,006,846 A *   | 12/1999 | Tibbitts et al. .... |
| 4,606,738 A   | 8/1986  | Hayden             | 6,009,963 A     | 1/2000  | Chaves et al.        |
| 4,621,031 A   | 11/1986 | Scruggs            | 6,050,354 A *   | 4/2000  | Pessier et al. ....  |
| 4,636,253 A   | 1/1987  | Nakai et al.       | 6,063,333 A     | 5/2000  | Dennis               |
| 4,645,977 A   | 2/1987  | Kurokawa et al.    | 6,123,612 A     | 9/2000  | Goers                |
| 4,662,348 A   | 5/1987  | Hall et al.        | 6,126,741 A     | 10/2000 | Jones et al.         |
| 4,664,705 A   | 5/1987  | Horton et al.      | 6,149,695 A *   | 11/2000 | Adia et al. ....     |
| 4,670,025 A   | 6/1987  | Pipkin             | 6,234,261 B1    | 5/2001  | Evans et al.         |
| 4,707,384 A   | 11/1987 | Schachner et al.   | 6,248,447 B1    | 6/2001  | Griffin et al.       |
| 4,726,718 A   | 2/1988  | Meskin et al.      | 6,269,894 B1    | 8/2001  | Griffin              |
| 4,766,040 A   | 8/1988  | Hillert et al.     | 6,332,503 B1 *  | 12/2001 | Pessier et al. ....  |
| 4,776,861 A   | 10/1988 | Frushour           | 6,344,149 B1    | 2/2002  | Oles                 |
| 4,784,023 A   | 11/1988 | Dennis             | 6,397,958 B1 *  | 6/2002  | Charles et al. ....  |
| 4,792,001 A   | 12/1988 | Zijssling          | 6,410,085 B1    | 6/2002  | Griffin et al.       |
| 4,793,828 A   | 12/1988 | Burnand            | 6,435,058 B1    | 8/2002  | Matthias et al.      |
| 4,797,241 A   | 1/1989  | Peterson et al.    | 6,544,308 B2 *  | 4/2003  | Griffin et al. ....  |
| 4,802,539 A   | 2/1989  | Hall et al.        | 6,592,985 B2 *  | 7/2003  | Griffin et al. ....  |
| 4,807,402 A   | 2/1989  | Rai                | 6,601,662 B2    | 8/2003  | Matthias et al.      |
| 4,828,582 A   | 5/1989  | Frushour           | 2005/0139397 A1 | 6/2005  | Achilles             |
| 4,844,185 A   | 7/1989  | Newton, Jr. et al. | 2007/0181348 A1 | 8/2007  | Lancaster et al.     |
| 4,861,350 A   | 8/1989  | Phaal et al.       |                 |         |                      |
| 4,871,377 A   | 10/1989 | Frushour           |                 |         |                      |
| 4,899,922 A   | 2/1990  | Slutz et al.       |                 |         |                      |
| 4,919,220 A   | 4/1990  | Fuller et al.      |                 |         |                      |
| 4,940,180 A   | 7/1990  | Martell            |                 |         |                      |
| 4,943,488 A   | 7/1990  | Sung et al.        |                 |         |                      |
| 4,944,772 A   | 7/1990  | Cho                |                 |         |                      |
| 4,976,324 A   | 12/1990 | Tibbitts           |                 |         |                      |
| 5,011,514 A   | 4/1991  | Cho et al.         |                 |         |                      |
| 5,027,912 A   | 7/1991  | Juergens           |                 |         |                      |
| 5,030,276 A   | 7/1991  | Sung et al.        |                 |         |                      |
| 5,092,687 A   | 3/1992  | Hall               |                 |         |                      |
| 5,116,568 A   | 5/1992  | Sung et al.        |                 |         |                      |
| 5,120,327 A * | 6/1992  | Dennis .....       | 407/119         |         |                      |
| 5,127,923 A   | 7/1992  | Bunting et al.     |                 |         |                      |
| 5,135,061 A   | 8/1992  | Newton, Jr.        |                 |         |                      |
| 5,176,720 A   | 1/1993  | Martell et al.     |                 |         |                      |
| 5,186,725 A   | 2/1993  | Martell et al.     |                 |         |                      |
| 5,199,832 A   | 4/1993  | Meskin et al.      |                 |         |                      |
| 5,205,684 A   | 4/1993  | Meskin et al.      |                 |         |                      |
| 5,213,248 A   | 5/1993  | Horton et al.      |                 |         |                      |
| 5,238,074 A   | 8/1993  | Tibbitts et al.    |                 |         |                      |
| 5,264,283 A   | 11/1993 | Waldenstrom        |                 |         |                      |
| 5,337,844 A   | 8/1994  | Tibbitts           |                 |         |                      |
| 5,370,195 A   | 12/1994 | Keshavan et al.    |                 |         |                      |
| 5,379,853 A   | 1/1995  | Lockwood           |                 |         |                      |
| 5,439,492 A   | 8/1995  | Anthony et al.     |                 |         |                      |
| 5,464,068 A   | 11/1995 | Najafi-Sani        |                 |         |                      |
| 5,468,268 A   | 11/1995 | Tank et al.        |                 |         |                      |
| 5,496,638 A   | 3/1996  | Waldenstrom        |                 |         |                      |
| 5,505,748 A   | 4/1996  | Tank et al.        |                 |         |                      |
| 5,510,193 A   | 4/1996  | Cerutti et al.     |                 |         |                      |
| 5,523,121 A   | 6/1996  | Anthony et al.     |                 |         |                      |

## FOREIGN PATENT DOCUMENTS

|    |                |         |
|----|----------------|---------|
| EP | 0329954        | 8/1993  |
| EP | 0617207        | 9/1994  |
| EP | 0585631        | 4/1997  |
| EP | 0787820        | 8/1997  |
| EP | 0500253        | 11/1997 |
| EP | 0595630        | 1/1998  |
| EP | 0612868        | 7/1998  |
| EP | 0860515        | 8/1998  |
| EP | 1 190 791 A2   | 3/2002  |
| EP | 1190791 A2     | 3/2002  |
| GB | 1349385        | 4/1974  |
| GB | 2048927        | 12/1980 |
| GB | 2268768        | 1/1994  |
| GB | 2323398        | 9/1998  |
| RU | 566439         | 1/2000  |
| RU | 2034937        | 9/2004  |
| WO | WO 93/23204    | 11/1993 |
| WO | WO 96/34131    | 10/1996 |
| WO | WO 00/28106    | 5/2000  |
| WO | WO 2004/040095 | 5/2004  |
| WO | WO 2004/106003 | 12/2004 |
| WO | WO 2004/106004 | 12/2004 |

## OTHER PUBLICATIONS

|                                                                         |
|-------------------------------------------------------------------------|
| Office Action dated Aug. 8, 2007 for related U.S. Appl. No. 11/022,271. |
| Office Action dated Apr. 3, 2007 for related U.S. Appl. No. 11/022,272. |
| Office Action dated Oct. 4, 2007 for related U.S. Appl. No. 11/022,272. |
| Office Action dated May 9, 2008, for related U.S. Appl. No. 11/022,271. |

Declaration of Stephen C. Steinke.

Declaration of John L. Williams.

Declaration of Anthony Griffo.

Declaration of Ronald K. Eyre.

Declaration of Stewart Middlemiss.

Examination Report for United Kingdom Application No. GB1001703.6, mailed on Feb. 25, 2010 (6 pages).

Examination Report for United Kingdom Application No. GB1001698.8, mailed on Feb. 25, 2010 (6 pages).

Examination Report for United Kingdom Application No. GB1001690.5, mailed on Feb. 25, 2010 (6 pages).

Examination Report for United Kingdom Application No. GB1001691.3, mailed on Feb. 25, 2010 (6 pages).

Examination Report for United Kingdom Application No. GB0519211.7, mailed on Nov. 17, 2009 (2 pages).

Examination Report for United Kingdom Application No. 0519211.7, mailed on Apr. 23, 2010 (2 pages).

\* cited by examiner



FIG. 1



FIG. 2B



FIG. 2A



FIG. 2C



FIG. 2D



FIG. 3



FIG. 2E



FIG. 4



**FIG. 5**



**FIG. 6**





FIG. 10



FIG. 11



*FIG. 12*

# THERMALLY STABLE DIAMOND POLYCRYSTALLINE DIAMOND CONSTRUCTIONS

## FIELD OF THE INVENTION

This invention generally relates to polycrystalline diamond materials and, more specifically, to polycrystalline diamond materials that have been specifically engineered to provide an improved degree of thermal stability when compared to conventional polycrystalline diamond materials, thereby providing an improved degree of service life in desired cutting and/or drilling applications.

## BACKGROUND OF THE INVENTION

Polycrystalline diamond (PCD) materials and PCD elements formed therefrom are well known in the art. Conventional PCD is formed by combining synthetic diamond grains with a suitable solvent catalyst material to form a mixture. The mixture is subjected to processing conditions of extremely high pressure/high temperature, where the solvent catalyst material promotes desired intercrystalline diamond-to-diamond bonding between the grains, thereby forming a PCD structure. The resulting PCD structure produces enhanced properties of wear resistance and hardness, making PCD materials extremely useful in aggressive wear and cutting applications where high levels of wear resistance and hardness are desired.

Solvent catalyst materials typically used for forming conventional PCD include metals from Group VIII of the Periodic table, with cobalt (Co) being the most common. Conventional PCD can comprise from 85 to 95% by volume diamond and a remaining amount solvent catalyst material. The material microstructure of conventional PCD comprises regions of intercrystalline bonded diamond with solvent catalyst material attached to the diamond and/or disposed within interstices or interstitial regions that exist between the intercrystalline bonded diamond regions.

A problem known to exist with such conventional PCD materials is that they are vulnerable to thermal degradation, when exposed to elevated temperature cutting and/or wear applications, caused by the differential that exists between the thermal expansion characteristics of the interstitial solvent metal catalyst material and the thermal expansion characteristics of the intercrystalline bonded diamond. Such differential thermal expansion is known to occur at temperatures of about 400° C., can cause ruptures to occur in the diamond-to-diamond bonding, and eventually result in the formation of cracks and chips in the PCD structure, rendering the PCD structure unsuited for further use.

Another form of thermal degradation known to exist with conventional PCD materials is one that is also related to the presence of the solvent metal catalyst in the interstitial regions and the adherence of the solvent metal catalyst to the diamond crystals. Specifically, the solvent metal catalyst is known to cause an undesired catalyzed phase transformation in diamond (converting it to carbon monoxide, carbon dioxide, or graphite) with increasing temperature, thereby limiting practical use of the PCD material to about 750° C.

Attempts at addressing such unwanted forms of thermal degradation in conventional PCD materials are known in the art. Generally, these attempts have focused on the formation of a PCD body having an improved degree of thermal stability when compared to the conventional PCD materials discussed above. One known technique of producing a PCD body hav-

ing improved thermal stability involves, after forming the PCD body, removing all or a portion of the solvent catalyst material therefrom.

For example, U.S. Pat. No. 6,544,308 discloses a PCD element having improved wear resistance comprising a diamond matrix body that is integrally bonded to a metallic substrate. While the diamond matrix body is formed using a catalyzing material during high temperature/high pressure processing, the diamond matrix body is subsequently treated to render a region extending from a working surface to a depth of at least about 0.1 mm substantially free of the catalyzing material, wherein 0.1 mm is described as being the critical depletion depth.

Japanese Published Patent Application 59-219500 discloses a diamond sintered body joined together with a cemented tungsten carbide base formed by high temperature/high pressure process, wherein the diamond sintered body comprises diamond and a ferrous metal binding phase. Subsequent to the formation of the diamond sintered body, a majority of the ferrous metal binding phase is removed from an area of at least 0.2 mm from a surface layer of the diamond sintered body.

In addition to the above-identified references that disclose treatment of the PCD body to improve the thermal stability by removing the catalyzing material from a region of the diamond body extending a minimum distance from the diamond body surface, there are other known references that disclose the practice of removing the catalyzing material from the entire PCD body. While this approach produces an entire PCD body that is substantially free of the solvent catalyst material, it is fairly time consuming. Additionally, a problem known to exist with this approach is that the lack of solvent metal catalyst within the PCD body precludes the subsequent attachment of a metallic substrate to the PCD body by solvent catalyst infiltration.

Additionally, PCD bodies rendered thermally stable by removing substantially all of the catalyzing material from the entire body have a coefficient of thermal expansion that is sufficiently different from that of conventional substrate materials (such as WC—Co and the like) that are typically infiltrated or otherwise attached to the PCD body. The attachment of such substrates to the PCD body is highly desired to provide a PCD compact that can be readily adapted for use in many desirable applications. However, the difference in thermal expansion between the thermally stable PCD body and the substrate, and the poor wettability of the thermally stable PCD body diamond surface due to the substantial absence of solvent metal catalyst, makes it very difficult to bond the thermally stable PCD body to conventionally used substrates. Accordingly, such PCD bodies must be attached or mounted directly to a device for use, i.e., without the presence of an adjoining substrate.

Since such PCD bodies, rendered thermally stable by having the catalyzing material removed from the entire diamond body, are devoid of a metallic substrate they cannot (e.g., when configured for use as a drill bit cutter) be attached to a drill bit by conventional brazing process. The use of such thermally stable PCD body in this particular application necessitates that the PCD body itself be mounted to the drill bit by mechanical or interference fit during manufacturing of the drill bit, which is labor intensive, time consuming, and does not provide a most secure method of attachment.

While these above-noted known approaches provide insight into diamond bonded constructions capable of providing some improved degree of thermal stability when compared to conventional PCD constructions, it is believed that further improvements in thermal stability for PCD materials

useful for desired cutting and wear applications can be obtained according to different approaches that are both capable of minimizing the amount of time and effort necessary to achieve the same, and that permit formation of a thermally stable PCD construction comprising a desired substrate bonded thereto to facilitate attachment of the construction with a desired application device.

It is, therefore, desired that diamond compact constructions be developed that include a PCD body having an improved degree of thermal stability when compared to conventional PCD materials, and that include a substrate material bonded to the PCD body to facilitate attachment of the resulting thermally stable compact construction to an application device by conventional method such as welding or brazing and the like. It is further desired that such a compact construction provide a desired degree of thermal stability in a manner that can be manufactured at reasonable cost without requiring excessive manufacturing times and without the use of exotic materials or techniques.

#### SUMMARY OF THE INVENTION

Thermally stable diamond constructions, prepared according to principles of this invention, comprise a diamond body having a plurality of bonded diamond crystals and a plurality of interstitial regions disposed among the crystals. A metallic substrate is attached to the diamond body.

The diamond body includes a working surface positioned along an outside portion of the body. The diamond body comprises a first region that is substantially free of a catalyst material, and a second region that includes the catalyst material. In an example embodiment, the diamond body first region extends from the working surface to depth of at least about 0.02 mm to a depth of less than about 0.09 mm.

In an example embodiment, the diamond body comprises diamond crystals having an average diamond grain size of greater than about 0.02 mm, and comprises at least 85 percent by volume diamond based on the total volume of the diamond body. Additionally, the second region can have an average thickness of at least about 0.01 mm, and the diamond body can be formed from natural diamond powder.

Thermally stable diamond constructions of this invention may be provided in the form of a compact comprising a polycrystalline diamond body attached to a substrate. The compact is treated so that a desired surface of the diamond body to be rendered thermally stable remains exposed therefrom, and so that the remaining portion of the diamond body and the substrate is protected. Protection of the remaining portion can be achieved by using a protective material, for example, provided in the form of a coating or a protective member. In a preferred embodiment, such protection is provided by the use of a protective member or fixture that is configured to provide a leak-tight seal with the compact. The compact and fixture form an assembly that is subjected to the desired treating agent, whereby the exposed surface of the diamond body is placed into contact with the treating agent for a predetermined period of time to provide a thermally stable region within the diamond body extending a desired depth beneath the working surface.

Thermally stable constructions of this invention display an enhanced degree of thermal stability when compared to conventional PCD materials, and include a substrate material bonded to the PCD body that facilitates attachment therewith

to an application device by conventional method such as welding or brazing and the like.

#### BRIEF DESCRIPTION OF THE DRAWINGS

These and other features and advantages of the present invention will be appreciated as the same becomes better understood by reference to the following detailed description when considered in connection with the accompanying drawings wherein:

FIG. 1 is a schematic view of a region of polycrystalline diamond prepared in accordance with principals of this invention;

FIGS. 2A to 2E are perspective views of different polycrystalline diamond compacts of this invention comprising the region illustrated in FIG. 1;

FIG. 3 is a perspective view of an example embodiment thermally stable polycrystalline diamond construction of this invention;

FIG. 4 is a cross-sectional side view of the example embodiment thermally stable polycrystalline diamond construction of this invention as illustrated in FIG. 3;

FIG. 5 is a schematic view of a region of the thermally stable polycrystalline diamond construction of this invention;

FIG. 6 is a cross-sectional side view of a region of an example embodiment thermally stable polycrystalline diamond construction of this invention;

FIG. 7 is a perspective side view of an insert, for use in a roller cone or a hammer drill bit, comprising the thermally stable polycrystalline diamond construction of this invention;

FIG. 8 is a perspective side view of a roller cone drill bit comprising a number of the inserts of FIG. 7;

FIG. 9 is a perspective side view of a percussion or hammer bit comprising a number of inserts of FIG. 7;

FIG. 10 is a schematic perspective side view of a diamond shear cutter comprising the thermally stable polycrystalline diamond construction of this invention;

FIG. 11 is a perspective side view of a drag bit comprising a number of the shear cutters of FIG. 10; and

FIG. 12 is a cross-sectional perspective view of a protective fixture.

#### DETAILED DESCRIPTION

Thermally stable polycrystalline diamond (TSPCD) constructions of this invention are specifically engineered having a diamond bonded body comprising a region of thermally stable diamond extending a selected depth from a body working or cutting surface, thereby providing an improved degree of thermal stability when compared to conventional PCD materials not having such a thermally stable diamond region.

As used herein, the term "PCD" is used to refer to polycrystalline diamond that has been formed, at high pressure/high temperature (HPHT) conditions, through the use of a solvent metal catalyst, such as those included in Group VIII of the Periodic table. "Thermally stable polycrystalline diamond" as used herein is understood to refer to intercrystalline bonded diamond that includes a volume or region that has been rendered substantially free of the solvent metal catalyst used to form PCD, or the solvent metal catalyst used to form PCD remains in the region of the diamond body but is otherwise reacted or otherwise rendered ineffective in its ability adversely impact the bonded diamond at elevated temperatures as discussed above.

TSPCD constructions of this invention can further include a substrate attached to the diamond body that facilitates the attachment of the TSPCD construction to cutting or wear

devices, e.g., drill bits when the TSPCD construction is configured as a cutter, by conventional means such as by brazing and the like.

FIG. 1 illustrates a region of PCD **10** formed during a high pressure/high temperature (HPHT) process stage of forming this invention. The PCD has a material microstructure comprising a material phase of intercrystalline diamond made up of a plurality of bonded together adjacent diamond grains **12** at HPHT conditions. The PCD material microstructure also includes interstitial regions **14** disposed between bonded together adjacent diamond grains. During the HPHT process, the solvent metal catalyst used to facilitate the bonding together of the diamond grains migrates into and resides within these interstitial regions **14**.

FIG. 2A illustrates an example PCD compact **16** formed in accordance with this invention by HPHT process. The PCD compact **16** generally comprises a PCD body **18**, having the material microstructure described above and illustrated in FIG. 1, that is bonded to a desired substrate **20**. Although the PCD compact **16** is illustrated as being generally cylindrical in shape and having a disk-shaped flat or planar surface **22**, it is understood that this is but one preferred embodiment and that the PCD body as used with this invention can be configured other than as specifically disclosed or illustrated. It is further to be understood that the compact **16** may be configured having working or cutting surfaces disposed along the disk-shaped surface and/or along side surfaces **24** of the PCD body, depending on the particular cutting or wear application. Alternatively, the PCD compact may be configured having an altogether different shape but generally comprising a substrate and a PCD body bonded to the substrate, wherein the PCD body is provided with working or cutting surfaces oriented as necessary to perform working or cutting service when the compact is mounted to a desired drilling or cutting device, e.g., a drill bit.

FIGS. 2B to 2D illustrate alternative embodiments of PCD compacts of this invention having a substrate and/or PCD body configured differently than that illustrated in FIG. 2A. For example, FIG. 2B illustrates a PCD compact **16** configured in the shape of a preflat or gage trimmer including a cut-off portion **19** of the PCD body **18** and the substrate **20**. The preflat includes working or cutting surface positioned along a disk-shaped surface **22** and a side surface **24** working surface. Alternative preflat or gage trimmer PCD compact configurations intended to be within the scope of this invention include those described in U.S. Pat. No. 6,604,588, which is incorporated herein by reference.

FIG. 2C illustrates another embodiment of a PCD compact **16** of this invention configured having the PCD body **18** disposed onto an angled underlying surface of the substrate **20** and having a disk-shaped surface **22** that is the working surface and that is positioned at an angle relative to an axis of the compact. FIG. 2D illustrates another embodiment of a PCD compact **16** of this invention configured having the substrate **20** and the PCD body **18** disposed onto a surface of the substrate. In this particular embodiment, the PCD body has a domed or convex surface **22** serving as the working surface **22** (similar to the PCD compact embodiment described below and illustrated in FIG. 7).

FIG. 2E illustrates a still other embodiment of a PCD compact **16** of this invention that is somewhat similar to that illustrated in FIG. 2A in that it includes a PCD body **18** disposed on the substrate **20** and having a disk-shaped surface **22** as a working surface. Unlike the embodiment of FIG. 2A, however, this PCD compact includes an interface **21** between the PCD body and the substrate that is not uniformly planar. In this particular example, the interface **21** is canted or oth-

erwise non-axially symmetric. It is to be understood that PCD compacts of this invention can be configured having PCD body-substrate interfaces that are uniformly planer or that are not uniformly planer in a manner that is symmetric or non-symmetric relative to an axis running through the compact. Examples of other configurations of PCD compacts having nonplanar PCD body-substrate interfaces include those described in U.S. Pat. No. 6,550,556, which is incorporated herein by reference.

10 Diamond grains useful for forming the PCD body of this invention during the HPHT process include diamond powders having an average diameter grain size in the range of from submicrometer in size to 0.1 mm, and more preferably in the range of from about 0.005 mm to 0.08 mm. The diamond powder can contain grains having a mono or multi-modal size distribution. In a preferred embodiment for a particular application, the diamond powder has an average particle grain size of approximately 20 to 25 micrometers. However, it is to be understood that the use of diamond grains having a grain size less than this amount, e.g., less than about 15 micrometers, is useful for certain drilling and/or cutting applications. In the event that diamond powders are used having differently sized grains, the diamond grains are mixed together by conventional process, such as by ball or attritor milling for as much time as necessary to ensure good uniform distribution.

15 The diamond powder used to prepare the PCD body can be synthetic diamond powder. Synthetic diamond powder is known to include small amounts of solvent metal catalyst material and other materials entrained within the diamond crystals themselves. Alternatively, the diamond powder used to prepare the PCD body can be natural diamond powder. Unlike synthetic diamond powder, natural diamond powder does not include such solvent metal catalyst material and other materials entrained within the diamond crystals. It is theorized that that inclusion of materials other than the solvent catalyst in the synthetic diamond powder can operate to impair or limit the extent to which the resulting PCD body can be rendered thermally stable, as these materials along with the solvent catalyst must also be removed or otherwise neutralized. Since natural diamond is largely devoid of these other materials, such materials do not have to be removed from the PCD body and a higher degree of thermal stability can thus be obtained. Accordingly, for applications calling for a high degree of thermal stability the use of natural diamond for forming the PCD body is preferred. The diamond grain powder, whether synthetic or natural, is combined with or already includes a desired amount of catalyst material to facilitate desired intercrystalline diamond bonding during HPHT processing. Suitable catalyst materials useful for forming the PCD body include those solvent metals selected from the Group VIII of the Periodic table, with cobalt (Co) being the most common, and mixtures or alloys of two or more of these materials. The diamond grain powder and catalyst material mixture can comprise 85 to 95% by volume diamond grain powder and the remaining amount catalyst material. Alternatively, the diamond grain powder can be used without adding a solvent metal catalyst in applications where the solvent metal catalyst can be provided by infiltration during HPHT processing from the adjacent substrate or adjacent other body to be bonded to the PCD body.

20 In certain applications it may be desired to have a PCD body comprising a single PCD-containing volume or region, while in other applications it may be desired that a PCD body be constructed having two or more different PCD-containing volumes or regions. For example, it may be desired that the PCD body include a first PCD-containing region extending a distance from a working surface, and a second PCD-contain-

ing region extending from the first PCD-containing region to the substrate. The PCD-containing regions can be formed having different diamond densities and/or be formed from different diamond grain sizes. It is, therefore, understood that TSPCD constructions of this invention may include one or multiple PCD regions within the PCD body as called for by a particular drilling or cutting application.

The diamond grain powder and catalyst material mixture is preferably cleaned, and loaded into a desired container for placement within a suitable HPHT consolidation and sintering device, and the device is then activated to subject the container to a desired HPHT condition to consolidate and sinter the diamond powder mixture to form PCD.

In an example embodiment, the device is controlled so that the container is subjected to a HPHT process comprising a pressure in the range of from 5 to 7 GPa and a temperature in the range of from about 1320 to 1600° C., for a sufficient period of time. During this HPHT process, the catalyst material in the mixture melts and infiltrates the diamond grain powder to facilitate intercrystalline diamond bonding. During the formation of such intercrystalline diamond bonding, the catalyst material migrates into the interstitial regions within the microstructure of the so-formed PCD body that exists between the diamond bonded grains (see FIG. 1).

The PCD body can be formed with or without having a substrate material bonded thereto. In the event that the formation of a PCD compact comprising a substrate bonded to the PCD body is desired, a selected substrate is loaded into the container adjacent the diamond powder mixture prior to HPHT processing. An advantage of forming a PCD compact having a substrate bonded thereto is that it enables attachment of the to-be-formed TSPCD construction to a desired wear or cutting device by conventional method, e.g., brazing or welding. Additionally, in the event that the PCD body is to be bonded to a substrate, and the substrate includes a metal solvent catalyst, the metal solvent catalyst needed for catalyzing intercrystalline bonding of the diamond can be provided by infiltration. In which case is may not be necessary to mix the diamond powder with a metal solvent catalyst prior to HPHT processing.

Suitable materials useful as substrates for forming PCD compacts of this invention include those conventionally used as substrates for conventional PCD compacts, such as those formed from metallic and cermet materials. In a preferred embodiment, the substrate is provided in a preformed state and includes a metal solvent catalyst that is capable of infiltrating into the adjacent diamond powder mixture during processing to facilitate and provide a bonded attachment therewith. Suitable metal solvent catalyst materials include those selected from Group VIII elements of the Periodic table. A particularly preferred metal solvent catalyst is cobalt (Co). In a preferred embodiment, the substrate material comprises cemented tungsten carbide (WC—Co).

Once formed, the PCD body or compact is treated to render a selected region thereof thermally stable. This can be done, for example, by removing substantially all of the catalyst material from the selected region by suitable process, e.g., by acid leaching, aqua regia bath, electrolytic process, or combinations thereof. Alternatively, rather than actually removing the catalyst material from the PCD body or compact, the selected region of the PCD body or compact can be rendered thermally stable by treating the catalyst material in a manner that reduces or eliminates the potential for the catalyst material to adversely impact the intercrystalline bonded diamond at elevated temperatures. For example, the catalyst material can be combined chemically with another material to cause it to no longer act as a catalyst material, or can be transformed

into another material that again causes it to no longer act as a catalyst material. Accordingly, as used herein, the terms “removing substantially all” or “substantially free” as used in reference to the catalyst material is intended to cover the different methods in which the catalyst material can be treated to no longer adversely impact the intercrystalline diamond in the PCD body or compact with increasing temperature.

It is desired that the selected thermally stable region for TSPCD constructions of this invention is one that extends a determined depth from a surface, e.g., a working or cutting surface, of the diamond body independent of the working or cutting surface orientation. Again, it is to be understood that the working or cutting surface may include more than one surface portion of the diamond body. In an example embodiment, it is desired that the thermally stable region extend from a working or cutting surface of the PCD body an average depth of at least about 0.008 mm to an average depth of less than about 0.1 mm, preferably extend from a working or cutting surface an average depth of from about 0.02 mm to an average depth of less than about 0.09 mm, and more preferably extend from a working or cutting surface an average depth of from about 0.04 mm to an average depth of about 0.08 mm. The exact depth of the thermally stable region can and will vary within these ranges for TSPCD constructions of this invention depending on the particular cutting and wear application.

Generally, it has been shown that thermally stable regions within these ranges of depth produce a TSPCD construction having improved properties of wear and abrasion resistance when compared to conventional PCD compacts, while also providing desired properties of fracture strength and toughness. It is believed that thermally stable regions having depths greater than the upper limits noted above, while possibly capable of exhibiting a higher degree of wear and abrasion resistance, would in fact be brittle and have reduced strength and toughness, for aggressive drilling and/or cutting applications, and for this reason would likely fail in application and exhibit a reduced service life due to premature spalling or chipping.

It is to be understood that the depth of the thermally stable region from the working or cutting surface is represented as being a nominal, average value arrived at by taking a number of measurements at preselected intervals along this region and then determining the average value for all of the points. The region remaining within the PCD body or compact beyond this thermally stable region is understood to still contain the catalyst material.

Additionally, when the PCD body to be treated includes a substrate, i.e., is provided in the form of a PCD compact, it is desired that the selected depth of the region to be rendered thermally stable be one that allows a sufficient depth of region remaining in the PCD compact that is untreated to not adversely impact the attachment or bond formed between the diamond body and the substrate, e.g., by solvent metal infiltration during the HPHT process. In an example PCD compact embodiment, it is desired that the untreated or remaining region within the diamond body have a thickness of at least about 0.01 mm as measured from the substrate. It is, however, understood that the exact thickness of the PCD region containing the catalyst material next to the substrate can and will vary depending on such factors as the size and configuration of the compact, i.e., the smaller the compact diameter the smaller the thickness, and the particular PCD compact application.

In an example embodiment, the selected region of the PCD body is rendered thermally stable by removing substantially all of the catalyst material therefrom by exposing the desired

surface or surfaces to acid leaching, as disclosed for example in U.S. Pat. No. 4,224,380, which is incorporated herein by reference. Generally, after the PCD body or compact is made by HPHT process, the identified surface or surfaces, e.g., the working or cutting surfaces, are placed into contact with the acid leaching agent for a sufficient period of time to produce the desired leaching or catalyst material depletion depth.

Suitable leaching agents for treating the selected region to be rendered thermally stable include materials selected from the group consisting of inorganic acids, organic acids, mixtures and derivatives thereof. The particular leaching agent that is selected can depend on such factors as the type of catalyst material used, and the type of other non-diamond metallic materials that may be present in the PCD body, e.g., when the PCD body is formed using synthetic diamond powder. While removal of the catalyst material from the selected region operates to improve the thermal stability of the selected region, it is known that PCD bodies especially formed from synthetic diamond powder can include, in addition to the catalyst material, other metallic elements that can also contribute to thermal instability.

For example, one of the primary metallic phases known to exist in the PCD body formed from synthetic diamond powder is tungsten. It is, therefore, desired that the leaching agent selected to treat the selected PCD body region be one capable of removing both the catalyst material and such other known metallic materials. In an example embodiment, suitable leaching agents include hydrofluoric acid (HF), hydrochloric acid (HCl), nitric acid ( $HNO_3$ ), and mixtures thereof.

In an example embodiment, where the diamond body to be treated is in the form of a PCD compact, the compact is prepared for treatment by protecting the substrate surface and other portions of the PCD body adjacent the desired treated region from contact (liquid or vapor) with the leaching agent. Methods of protecting the substrate surface include covering, coating or encapsulating the substrate and portion of PCD body with a suitable barrier member or material such as wax, plastic or the like.

Referring to FIG. 12, in a preferred embodiment, the compact substrate surface and portion of the diamond body is protected by using an acid-resistant fixture 106 that is specifically designed to encapsulate the desired surfaces of the substrate and diamond body. Specifically, the fixture 106 is configured having a cylindrical body 108 within an inside surface diameter 110 that is sized to fit concentrically around the outside surface 111 of the compact 113. The fixture inside surface 110 can include a groove 112 extending circumferentially therearound and that is positioned adjacent to an end 114 of the fixture. The groove is sized to accommodate placement of a seal 115, e.g., in the form of an elastomeric O-ring or the like, therein. Alternatively, the fixture can be configured without a groove and a suitable seal can simply be interposed between the opposed respective compact and fixture outside and inside diameter surfaces. When placed around the outside surface of the compact, the seal operates to provide a leak-tight seal between the compact and the fixture to prevent unwanted migration of the leaching agent therebetween.

In a preferred embodiment, the fixture 106 includes an opening 117 in its end that is axially opposed end 114. The opening operates both to prevent an unwanted build up of pressure within the fixture when the PCD compact is loaded therein (which pressure could operate to urge the compact away from its loaded position within the fixture), and to facilitate the removal of the compact from the fixture once the treatment process is completed (e.g., the opening provides an access port for pushing the compact out of the fixture by mechanical or pressure means). During the process of treating

the compact, the opening 117 is closed using a suitable seal element 119, e.g., in the form of a removable plug or the like.

In preparation for treatment, the fixture is positioned axially over the PCD compact and the compact is loaded into the fixture with the compact working surface directly outwardly towards the fixture end 114. The compact is then positioned within the fixture so that the compact working surface 121 projects a desired distance outwardly from sealed engagement with the fixture inside wall. Positioned in this manner within the fixture, the compact working surface 121 is freely exposed to make contact with the leaching agent via fixture opening 123 positioned at end 114.

The PCD compact 113 and fixture 106 form an assembly are then placed into a suitable container that includes a desired volume of the leaching agent 125. In a preferred embodiment, the level of the leaching agent within the container is such that the diamond body working surface 121 exposed within the fixture is completely immersed into the leaching agent. In a preferred embodiment, a sheet of perforated material 127, e.g., in the form of a mesh material that is chemically resistant to the leaching agent, can be placed within the container and interposed between the assembly and the container surface to provide a desired distance between the fixture and the container. The use of a perforated material ensures that, although it is in contact with the assembly, the leaching agent will be permitted to flow to the exposed compact working surface to produce the desired leaching result.

FIGS. 3 and 4 illustrate an embodiment of the TSPCD construction 26 of this invention after its has been treated to render a selected region of the PCD body thermally stable. The construction comprises a thermally stable region 28 that extends a selected depth "D" from a working or cutting surface 30 of the diamond body 32. The remaining region 34 of the diamond body 32 extending from the thermally stable region 28 to the substrate 36 comprises PCD having the catalyst material intact. In a first example embodiment, the thermally stable region extends a depth of approximately 0.045 mm from the working or cutting surface. In a second example embodiment, the thermally stable region extends a depth of approximately 0.075 mm from the working or cutting surface. Again, it is to be understood that the exact depth of the thermally stable region can and will vary within the ranges noted above depending on the particular end use drilling and/or cutting applications.

Additionally, as mentioned briefly above, it is to be understood that the TSPCD construction described above and illustrated in FIGS. 3 and 4 are representative of a single embodiment of this invention for purposes of reference, and that TSPCD constructions other than that specifically described and illustrated are within the scope of this invention. For example, TSPCD constructions comprising a diamond body having a thermally stable region and then two or more other regions are possible, wherein a region interposed between the thermally stable region and the region adjacent the substrate may be a transition region having a diamond density and/or formed from diamond grains sized differently from that of the other diamond-containing regions.

FIG. 5 illustrates the material microstructure 38 of the TSPCD construction of this invention and, more specifically, a section of the thermally stable region of the TSPCD construction. The thermally stable region comprises the inter-crystalline bonded diamond made up of the plurality of bonded together diamond grains 40, and a matrix of interstitial regions 42 between the diamond grains that are now substantially free of the catalyst material. The thermally stable region comprising the interstitial regions free of the

## 11

catalyst material is shown to extend a distance "D" from a working or cutting surface 44 of the TSPCD construction. In an example embodiment, the distance "D" is identified and measured by cross sectioning a TSPCD construction and using a sufficient level of magnification to identify the interface between the first and second regions. As illustrated in FIG. 5, the interface is generally identified as the location within the diamond body where a sufficient population of the catalyst material 46 is shown to reside within the interstitial regions.

The so-formed thermally stable region of TSPCD constructions of this invention is not subject to the thermal degradation encountered in the remaining areas of the PCD diamond body, resulting in improved thermal characteristics. The remaining region of the diamond body extending from depth "D" has a material microstructure that comprises PCD, as described above and illustrated in FIG. 1, that includes catalyst material 46 disposed within the interstitial regions.

As noted above, the location of the working or cutting surface for TSPCD constructions of this invention can and will vary depending on the particular cutting or wear application. In an example embodiment, the wear or cutting surface can extend beyond the upper surface of the construction embodiment illustrated in FIG. 2. For example, FIG. 6 illustrates an example embodiment TSPCD construction of this invention comprising a working surface 50 that extends from a substantially planar upper surface 52 of the construction to a beveled surface 54 that defines a circumferential edge of the upper surface. In this embodiment, the thermally stable region 56 extends the selected depth into the diamond body 57 from each of the upper and beveled surfaces 52 and 54.

In such embodiment, prior to treating the PCD compact to render the selected region thermally stable, the PCD compact is formed to have such working surfaces, i.e., is formed by machine process or the like to provide the desired the beveled surface 54. Thus, a feature of TSPCD constructions of this invention is that they include working or cutting surfaces, independent of location or orientation, having a thermally stable region extending a predetermined depth into the diamond body.

For certain applications, it has been discovered than an improved degree of thermal stability can be realized by extending the thermally stable region beyond the working surface of the construction, i.e., by rendering a surface portion other than but adjacent to the working or cutting surface thermally stable. As illustrated in FIG. 6, the thermally stable region 56 has been extended along an outer surface portion 58 of the construction that extends axially away from the beveled surface 54 along a side surface of the diamond body towards the substrate 60. In the example embodiment illustrated in FIG. 6, the thermally stable region 56 extends along only a partial length of the side surface and the length of the thermally stable region 56 along the side surface is greater than the depth of the first region 56 at the upper or top surface 52. While this surface portion 58 may not actually be placed into wear or cutting contact, the presence of the thermally stable region adjacent the beveled surface 54 that is placed into wear or cutting service operates to provide an enhanced degree of thermal stability to the construction. This is believed to occur because the enhanced thermal conductivity provided by the thermally stable surface portion that operates to help conduct heat away from the adjacent the working surface, thereby increasing the TSPCD construction thermal resistance and service life.

In an example embodiment, where the TSPCD construction is provided in the form of a cutting element for use in a drill bit, and the cutting element includes a beveled transition

## 12

between an upper working surface and a side outer surface, the thermally stable region may be extended axially from the beveled surface along the side surface for a distance that will vary depending on the particular construction size and application, but that will be sufficient to provide a desired degree of thermal conductivity enhancement to improve overall thermal stability of the construction.

While the feature of forming a thermally stable region, adjacent a working or cutting surface, from a portion of the PCD body that may not be placed into working or cutting contact has been described in the context of placement adjacent a beveled working surface, it is to be understood that according to the practice of this invention that such extended thermally stable regions can be used in conjunction with working or cutting surfaces of any configuration, orientation or placement on the TSPCD construction.

The above-described TSPCD constructions formed according to this invention will be better understood with reference to the following examples:

20 Synthetic diamond powder having an average grain size of approximately 20 micrometers was mixed together for a period of approximately 1 hour by conventional process. The resulting mixture included approximately six percent by volume cobalt solvent metal catalyst, and WC-Co based on the total volume of the mixture, and was cleaned. The mixture was loaded into a refractory metal container with a cemented tungsten carbide substrate and the container was surrounded by pressed salt (NaCl) and this arrangement was placed within a graphite heating element. This graphite heating element containing the pressed salt and the diamond powder/substrate encapsulated in the refractory container was then loaded in a vessel made of a high-temperature/high-pressure self-sealing powdered ceramic material formed by cold pressing into a suitable shape. The self-sealing powdered ceramic vessel was placed in a hydraulic press having one or more rams that press anvils into a central cavity. The press was operated to impose a pressure and temperature condition of approximately 5,500 MPa and approximately 1450° C. on the vessel for a period of approximately 20 minutes.

25 During this HPHT processing, the cobalt solvent metal catalyst infiltrated through the diamond powder and catalyzed intercrystalline diamond-to-diamond bonding to form a PCD body having a material microstructure as discussed above and illustrated in FIG. 1. Additionally, the solvent metal catalyst in the substrate infiltrated into the diamond powder mixture to form a bonded attachment with the PCD body, thereby resulting in the formation of a PCD compact. The container was removed from the device, and the resulting PCD compact was removed from the container. Prior to leaching, the PCD compact was finished machined and ground to achieve the desired compact finished dimensions, size and configuration. The resulting PCD compact had a diameter of approximately 16 mm, the PCD diamond body had a thickness of approximately 3 mm, and the substrate had a thickness of approximately 13 mm. The PCD compact had a beveled surface defining a circumferential edge of the upper surface. The PCD compact had a working or cutting surface defined by the upper surface and the beveled edge and a side surface.

30 A protective fixture as described above was placed concentrically around the outside surface of the compact to cover the substrate and a portion of the diamond body. The fixture was formed from a plastic material capable of surviving exposure

to the leaching agent, and included an elastomeric O-ring disposed circumferentially therein around an inside fixture surface adjacent an end of the fixture. The fixture was positioned over the compact so that a portion of the diamond body desired to be rendered thermally stable was exposed therefrom. The O-ring provided a desired seal between the PCD compact and fixture. The PCD compact and fixture assembly was placed with the compact exposed portion immersed into a volume of leaching agent disposed within a suitable container. The leaching agent was a mixture of HF and HNO<sub>3</sub> that was provided at a temperature of approximately 22° C.

The depth that the PCD compact was immersed into the leaching agent was a depth sufficient to provide a thermally stable region along the portion of the diamond body comprising the working surfaces, including the upper surface and beveled surface for this particular example. As noted above, if desired, the depth of immersion can be deeper to extend beyond the beveled surface to include a portion of the PCD body side surface extending from the working or cutting surfaces. In this example, the immersion depth was approximately 4 mm. The PCD compact was immersed on the leaching agent for a period of approximately 150 minutes. After the designated treatment time had passed, the PCD compact and fixture assembly were removed from the leaching agent and the compact was removed from the protective fixture.

It is to be understood that the time period for leaching to achieve a desired thermally stable region according to the practice of this invention can and will vary depending on a number of factors, such as the diamond volume density, the diamond grain size, the leaching agent, and the temperature of the leaching agent.

The resulting TSPCD construction formed according to this example had a thermally stable region that extended from the working surfaces a distance into the diamond body of approximately 0.045 mm.

#### Example 2

##### TSPCD Construction

A TSPCD construction of this invention was prepared according to the process described above for example 1 except that the treatment for providing a thermally stable region in the PCD body was conducted for longer period of time. Specifically, the PCD compact was immersed on the leaching agent for a period of approximately 300 minutes. After the designated treatment time had passed, the PCD compact and fixture assembly was removed from the leaching agent and PCD compact was removed from the protective fixture. The resulting TSPCD construction formed according to this example had a thermally stable region that extended from the working surfaces a distance into the diamond body of approximately 0.075 mm.

A feature of TSPCD constructions of this invention is that they include a defined thermally stable region within a PCD body that provides an improved degree of wear and abrasion resistance, when compared to conventional PCD, while at the same time providing a desired degree of strength and toughness unique to conventional PCD that has been rendered thermally stable by either removing the catalyst material from a more substantial portion of the diamond body or by removing the catalyst material entirely therefrom. A further feature of TSPCD constructions of this invention is that they include a thermally stable region that not only extends a determined depth from identified working surfaces, e.g., extending along both the upper and beveled compact surfaces, but that can include a further thermally stable region that positioned adja-

cent an identified working surface or surfaces, thereby operating to provide a further enhanced degree of thermal stability and resistance during cutting and/or wear service.

A further feature of TSPCD constructions of this invention is that they can be formed from natural diamond that, unlike synthetic diamond, does not include metallic impurities in the diamond grains that can otherwise limit the extent to which optimal thermal stability can be achieved by the treatment techniques described above. Accordingly, in certain applications calling for a high degree of thermally stability, the use of natural diamond can be used to achieve this result.

A still further feature of TSPCD constructions of this invention is that the thermally stable region is formed in a manner that does not adversely impact the compact substrate. Specifically, the treatment process is carefully controlled to ensure that a sufficient region within the PCD body adjacent the substrate remains unaffected and includes the catalyst material, thereby ensuring that the desired bond between the substrate and PCD body remain intact. Additionally, during the treatment process, means are used to protect the surface of the substrate from liquid or vapor contact with the leaching agent, to ensure that the substrate is in no way adversely impacted by the treatment.

A still further feature of TSPCD constructions of this invention is that they are provided in the form of a compact comprising a PCD body, having a thermally stable region, which body is bonded to a metallic substrate. This enables TSPCD constructions of this invention to be attached with different types of well known cutting and wear devices such as drill bits and the like by conventional attachment techniques such as by brazing or welding.

TSPCD constructions of this invention can be used in a number of different applications, such as tools for mining, cutting, machining and construction applications, where the combined properties of thermal stability, wear and abrasion resistance, and strength and toughness are highly desired. TSPCD constructions of this invention are particularly well suited for forming working, wear and/or cutting components in machine tools and drill and mining bits such as roller cone rock bits, percussion or hammer bits, diamond bits, and shear cutters.

FIG. 7 illustrates an embodiment of a TSPCD construction of this invention provided in the form of an insert 62 used in a wear or cutting application in a roller cone drill bit or percussion or hammer drill bit. For example, such TSPCD inserts 62 are constructed having a substrate portion 64, formed from one or more of the substrate materials disclosed above, that is attached to a PCD body 66 having a thermally stable region. In this particular embodiment, the insert comprises a domed working surface 68, and the thermally stable region is positioned along the working surface and extends a selected depth therefrom into the diamond body. The insert can be pressed or machined into the desired shape or configuration prior to the treatment for rendering the selected region thermally stable. It is to be understood that TSPCD constructions can be used with inserts having geometries other than that specifically described above and illustrated in FIG. 7.

FIG. 8 illustrates a rotary or roller cone drill bit in the form of a rock bit 70 comprising a number of the wear or cutting TSPCD inserts 72 disclosed above and illustrated in FIG. 7. The rock bit 70 comprises a body 74 having three legs 76 extending therefrom, and a roller cutter cone 78 mounted on a lower end of each leg. The inserts 72 are the same as those described above comprising the TSPCD constructions of this invention, and are provided in the surfaces of each cutter cone 78 for bearing on a rock formation being drilled.

## 15

FIG. 9 illustrates the TSPCD insert described above and illustrated in FIG. 7 as used with a percussion or hammer bit 80. The hammer bit generally comprises a hollow steel body 82 having a threaded pin 84 on an end of the body for assembling the bit onto a drill string (not shown) for drilling oil wells and the like. A plurality of the inserts 86 are provided in the surface of a head 88 of the body 82 for bearing on the subterranean formation being drilled.

FIG. 10 illustrates a TSPCD construction of this invention as embodied in the form of a shear cutter 90 used, for example, with a drag bit for drilling subterranean formations. The TSPCD shear cutter comprises a PCD body 92 that is sintered or otherwise attached to a cutter substrate 94 as described above. The PCD body includes a working or cutting surface 96 that is formed from the thermally stable region of the PCD body. As discussed and illustrated above, the working or cutting surface for the shear cutter can extend from the upper surface to a beveled surface defining a circumferential edge of the upper, and the thermally stable region of the PCD body can extend a depth from such working surfaces. Additionally, if desired, the thermally stable region of the PCD body can extend from the beveled or other working surface a distance axially along a side surface of the shear cutter to provide an enhanced degree of thermal stability and thermal resistance to the cutter. It is to be understood that TSPCD constructions can be used with shear cutters having geometries other than that specifically described above and illustrated in FIG. 10.

FIG. 11 illustrates a drag bit 98 comprising a plurality of the TSPCD shear cutters 100 described above and illustrated in FIG. 10. The shear cutters are each attached to blades 102 that extend from a head 104 of the drag bit for cutting against the subterranean formation being drilled. Because the TSPCD shear cutters of this invention include a metallic substrate, they are attached to the blades by conventional method, such as by brazing or welding.

Other modifications and variations of TSPCD constructions as practiced according to the principles of this invention will be apparent to those skilled in the art. It is, therefore, to be understood that within the scope of the appended claims, this invention may be practiced otherwise than as specifically described.

What is claimed is:

1. A thermally stable diamond construction comprising: a diamond body comprising a plurality of intercrystalline bonded diamond crystals, and a plurality of interstitial regions disposed among the crystals, the diamond body including:
  - an upper surface positioned along an outside portion of the body;
  - a thermally stable first region that is substantially free of a catalyst material in the interstitial regions; and
  - a second region that includes the catalyst material in the interstitial regions;
 wherein the first region extends from the upper surface to a depth of at least about 0.02 mm to less than about 0.09 mm;
2. The construction as recited in claim 1 wherein the second region is interposed between the first region and the metallic substrate.
3. The construction as recited in claim 1 wherein the first region extends from the upper surface to a depth of at least about 0.04 mm to about 0.08 mm.

## 16

4. The construction as recited in claim 1 wherein the upper surface extends along a side surface of the diamond body.

5. The construction as recited in claim 1 wherein the diamond body includes two or more surfaces that are oriented at different angles from one another on the diamond body.

6. The construction as recited in claim 1 wherein the diamond crystals have an average diamond grain size of greater than about 0.02 mm.

7. The construction as recited in claim 1 wherein the diamond body comprises at least 85 percent by volume diamond based on the total volume of the diamond body.

8. The construction as recited in claim 1 wherein the second region has an average thickness of at least about 0.01 mm.

9. The construction as recited in claim 1 wherein the diamond body is formed from natural diamond powder.

## 10. A cutting element comprising:

a diamond body comprising a plurality of intercrystalline bonded diamond crystals and a plurality of interstitial regions disposed among the crystals, the diamond body including:

at least one surface positioned along an outside portion of the body comprising a beveled peripheral edge interposed between a diamond body upper surface and a side surface;

a thermally stable first region that is substantially free of a catalyst material in the interstitial regions and that extends from the at least one surface to a depth that is greater than about 0.04 mm and less than about 0.08 mm; and

a second region extending from the first region that includes the catalyst material in the interstitial regions;

a metallic substrate attached to the diamond body.

11. The cutting element as recited in claim 10 wherein the diamond crystals have an average diamond grain size of greater than about 0.02 mm.

12. The cutting element as recited in claim 11 wherein the diamond body comprises at least 85 percent by volume diamond based on the total volume of the diamond body.

13. A thermally stable diamond construction prepared by the process of:

treating a polycrystalline diamond compact comprising a polycrystalline diamond body and a metallic substrate attached thereto, the polycrystalline diamond body having an upper surface and comprising a plurality of intercrystalline bonded diamond grains and interstitial regions disposed therebetween wherein the diamond body comprises 85 percent to 95 percent by volume of diamond crystals, to remove a catalyst material in the interstitial regions from a first region of the diamond body extending from the upper surface while allowing the catalyst material to remain in the interstitial regions in a second region of the diamond body;

wherein prior to the step of treating, protecting the metallic substrate from exposure to a treating agent used during the step of treating; and

wherein during the step of treating, controlling the depth of the first region so that it extends from the upper surface to a depth of not less than about 0.02 mm to a depth of not greater than about 0.09 mm.

14. The construction as recited in claim 1 wherein the upper surface is an outermost surface of the body element.

15. The construction as recited in claim 4 wherein the diamond body includes a beveled peripheral edge disposed along a circumferential edge of the upper surface.

## 17

16. The construction as recited in claim 4 wherein the first region extends along the side surface a partial length of the diamond body.

17. The construction as recited in claim 16 wherein the first region extending along the side surface extends a length along the body that is greater than the depth of the first region measured perpendicular to the upper surface.

18. The construction as recited in claim 1 wherein the includes a beveled peripheral edge disposed along a circumferential edge of the upper surface.

19. The construction as recited in claim 18 wherein the depth of the first region is approximately the same along the diamond body upper and beveled edge surfaces.

20. The construction as recited in claim 10 wherein the depth of the first region in the upper surface and beveled peripheral edge are approximately the same.

21. The cutting element as cited in claim 10 wherein the first region extends along a partial length of the diamond body side surface from the beveled edge.

22. The cutting element as recited in claim 21 wherein the first region extends along the side surface a length that exceeds the depth of the first region as measured perpendicular to side surface.

23. A thermally stable diamond construction comprising:  
a substrate; and  
a diamond body attached to the substrate and comprising a plurality of intercrystalline bonded diamond crystals and a plurality of interstitial regions disposed among the bonded diamond crystals,

the diamond body including an upper surface, a side surface extending away from the upper surface, and a beveled peripheral edge interposed between a diamond body upper surface and a side surface, and

the diamond body comprising:  
a first region of the diamond body extending from at least a portion of the upper surface a partial depth ranging from about 0.02 to 0.09 mm into the diamond body, along a portion of the side surface a partial depth into the diamond body, and along the beveled peripheral edge a partial depth into the diamond body, the first region being substantially free of a catalyst material in the interstitial regions; and

a second region adjacent the first region, the second region comprising the catalyst material in the interstitial regions.

24. The thermally stable diamond construction of claim 23, wherein the partial depth ranges from about 0.04 to 0.08 mm.

25. The thermally stable diamond construction of claim 23, wherein the second region is interposed between the first region and the substrate.

26. The thermally stable diamond construction of claim 23, wherein the first region extends a partial depth of at least 0.02 mm to less than about 0.09 mm from the portion of the side surface.

## 18

27. The thermally stable diamond construction of claim 23, wherein diamond body includes a beveled surface disposed along a circumferential edge of the upper surface.

28. The thermally stable diamond construction of claim 23, wherein the diamond crystals have an average diamond grain size of greater than about 0.02 mm.

29. The thermally stable diamond construction of claim 23, wherein the diamond body comprises at least 85 percent by volume diamond based on the total volume of the diamond body.

30. The thermally stable diamond construction of claim 23, wherein the second region has an average thickness of at least about 0.01 mm.

31. A thermally stable diamond construction comprising:  
a substrate; and

a diamond body attached to the substrate and comprising a plurality of bonded diamond crystals and a plurality of interstitial regions disposed among the bonded diamond crystals,

the diamond body including an upper surface and a side surface extending away from the upper surface, and the diamond body comprising:

a first region of the diamond body being substantially free of a catalyst material, and the first region extending into the diamond body from the upper surface a partial depth between about 0.02 mm and 0.09 mm and a partial depth along a partial length of the side surface, wherein the partial length extends along at least 50% of the side surface; and

a second region adjacent the first region, the second region comprising the catalyst material.

32. The thermally stable diamond construction of claim 31, wherein the partial depth from the upper surface ranges from about 0.04 to 0.08 mm.

33. The thermally stable diamond construction of claim 31, wherein the partial depth from the side surface ranges from about 0.02 to 0.09 mm.

34. The thermally stable diamond construction of claim 33, wherein the partial depth from the side surface ranges from about 0.04 to 0.08 mm.

35. The thermally stable diamond construction of claim 31, wherein the second region is interposed between the first region and the substrate.

36. The thermally stable diamond construction of claim 31, wherein diamond body comprises a beveled surface disposed along a circumferential edge of the upper surface.

37. The thermally stable diamond construction of claim 31, wherein the interstitial regions in the first region as substantially empty.

\* \* \* \* \*